

March 4, 1958

J. B. GERGEN ET AL

2,825,282

LETTERPRESS PRINTING MAKEREADY

Filed April 2, 1956



INVENTORS

JAMES B. GERGEN

THOMAS G. WARTMAN

BY  
Carpenter, Abbott, Coulter, & Kinney

ATTORNEYS

1

2,825,282

**LETTERPRESS PRINTING MAKEREADY**

James B. Gergen, West St. Paul, and Thomas G. Wartman, St. Paul, Minn., assignors to Minnesota Mining & Manufacturing Company, St. Paul, Minn., a corporation of Delaware

Application April 2, 1956, Serial No. 575,602

29 Claims. (Cl. 101—401.3)

This invention relates to the art of makeready especially as related to letterpress printing, to novel makeready methods and constructions, and to novel sheet material applicable thereto.

This application is a continuation-in-part of our application filed August 25, 1954, Serial No. 452,206, now abandoned.

In letterpress printing, including flat-bed as well as rotary press printing, an impression cylinder or platen is commonly used to press a sheet, usually paper, against the inked face (e. g., figures, designs, type, pictures, etc.) of a printing form. The face or image of the printing form (i. e., the surface of raised printing elements) is thereby printed upon the sheet.

Many different types or styles of apparatus may be used in this printing operation. Printing forms may be mounted so as to rest upon wood, honeycomb, or other types of bases. Impression cylinders or platens may be wrapped with several layers of "packing" materials, such as papers, cloths, draw sheets, etc. A suitable, but not necessarily exact, pitch or printing line is maintained for the operation. In describing this invention, all illustrations are taken with respect to flat-bed press printing using an impression cylinder, but it is understood that the teachings herein are not limited to any particular style of apparatus and that equivalent printing apparatus is equally suitable to employ.

For highest quality letterpress printing, certain preliminary steps are required in readying the printing apparatus for operation. Makeready is a part of this procedure and, as used herein, involves selectively varying the thickness of packing on various areas of an impression cylinder, and/or adjusting the height of, or packing beneath, various areas of the face on a printing form so that the impression pressure under which areas of the cylinder and areas of the face of the printing form coat during printing is selectively adjusted.

Prior art methods of makeready are extremely time consuming, costly, and, for the most part, do not readily give results comparable to the high quality obtained by the practice of this invention. They frequently require the use of messy materials, e. g., sticky ink, various powdery materials, etc., and in addition, individually suffer various other defects.

Among printers, the oldest known method of makeready, viz., the use of paper cutouts, dollies, etc., is the most popular. It has also been used to compensate for press irregularities. While the method is susceptible of producing excellent results, it is very time-consuming and results obtained are entirely dependent upon the skill and technique of the printer.

This invention to a large extent alleviates the burden and expense of makeready and provides a new method for accomplishing it expeditiously, accurately, economically and mechanically, all as will be evident as this description proceeds. By the practice of this invention, makeready is accomplished with a high degree of fidelity

2

and in a manner which permits a number of printing establishments required to print the same subject matter at various locations to duplicate easily the precise corrections necessary.

5 Further provided by this invention are convenient makeready sheet materials which mechanically expand in selective fashion when processed according to the teachings herein, which have desired strength and toughness in selectively expanded areas, and which may be stored in 10 the unexpanded state under ordinary atmospheric conditions without loss of their desired physical properties. These new sheet materials require no meticulous cutting for makeready use and permit makeready to be accomplished expeditiously and free of messy components, such 15 as pastes, powders, etc., as required in the prior art. We know of no makeready sheet materials of this type which were commercially available prior to our invention.

By utilizing the makeready teachings herein, prints may be made which have delicate shadings, dense solids and 20 clean highlights. Such prints, obtainable after only a short makeready time, are especially desired by publishers of encyclopedias, art magazines, and the like, where makeready has become an extremely time-consuming process. The various makeready constructions hereof give to printing 25 forms a longer press life than heretofore experienced.

In describing our invention, we choose to refer specifically to makeready for graphic arts printing forms, but it will be understood that our novel process and sheet materials are also suitable to employ in making ready, or as makeready for, other printing forms.

Fundamentally, theoretical explanations aside, to provide appropriately corrected impression pressures for highest quality graphic arts printing, the relative thickness of packing over solid tone areas must, with respect to the 30 thickness of packing over middletone areas, be increased.

Additionally, however, the thickness of packing over the peripheral area of solid tones generally should be less than that over central areas thereof, and further, the thickness of packing over middletone areas having a very high 35 density of dots or printing elements should be comparatively greater than that packing over middletone areas having a very low density of dots or printing elements. Of course, as evident from the above, the relative height of, or packing beneath, areas of solid tone may be raised or increased relatively to areas of middletone to accomplish 40 also a suitable correction for printing. Highlight or non-printing areas of a printing form should receive least pressure in printing and therefore should generally have the least packing.

50 Variation of the thickness of packing on an impression cylinder involves "overlay" makeready. Corrective material inserted beneath the mounting block on which a printing form rests is "underlay" makeready. "Interlay" makeready involves placing corrective material beneath 55 the printing form, e. g., an electrotype, but above the mounting block on which it rests. Adjusting the height of various areas on the face of a printing form may involve a "bump-up" process such as hereinafter described.

According to our invention, a makeready sheet material 60 having a flexible selectively-thermoeexpansive layer which is resistant to compression in expanded condition, is inked or printed with the general likeness of a printing form, exposed to radiant energy for differential sustained expansion, and finally, placed in registration with a printing form. The processed sheet material essentially provides the amount and kind of makeready correction needed to accomplish highest quality printing.

To illustrate the invention, but not limit the same, a 70 number of drawings are set forth wherein:

Figure 1 is a diagrammatic section through a makeready sheet hereof.

Figure 2 is a diagrammatic section through a portion of a printing form and an impression cylinder wrapped with our makeready sheet.

Figure 3 is a diagrammatic section through a source of high-intensity radiant energy and a makeready sheet selectively expanded in part.

Figure 4 is a diagrammatic section through a portion of a printing form and an impression cylinder having a selectively-expanded makeready sheet in registered overlay position.

Figure 5 is a diagrammatic exploded sectional view illustrating two squeeze rollers, two metal plates, and a laminate comprising a negative selectively expanded makeready sheet, a printing form, and a positive selectively expanded makeready sheet (here shown slightly out of register).

According to the preferred embodiment of our process, designated for brevity as the overlay process, the selectively-thermoexpansible layer or side of an overlay-type makeready sheet non-absorptive of radiant energy, e. g., a sheet such as illustrated in Figure 1 comprising a carrier web 20 and a selectively-thermoexpansible layer 21, is first inked or printed upon with a radiant energy absorptive ink. This may be accomplished in the manner illustrated in Figure 2. Sheet 22 with its heat-sensitive layer 21 outermost is fastened around impression cylinder 23 over several layers of packing 24, which provides adequate overall general impression pressure. Printing form 25, e. g., an electrotype, supported on mounting block 26, is inked and the wrapped impression cylinder rolled thereover. Desirably, the position of the resulting printed sheet on the impression cylinder is now marked, suitably by punching a few holes through the leading or front edge of the sheet and several layers of cylinder packing, so as to facilitate its subsequent registration.

After initial printing, the makeready sheet is removed from the impression cylinder and briefly exposed to uniform and intense radiant energy. Figure 3 illustrates one way for accomplishing suitable exposure. In this figure, sheet material 22 with inked layer 21 toward high-intensity radiation source 27 in elliptical reflector 28, is moved to the right, as indicated by the arrow, through narrow focused band 29 of radiant energy. In those areas to the right of band 29, the sheet is illustrated as selectively expanded according to the pattern of infrared absorption shown as inked thereon. Solid tone printed area 30 is greatly expanded, while middletone printed areas 31 and 32 of proportionately less printing point density are expanded only to a degree approximately commensurate with their tone. Unexpanded printed areas 33, to the left of the focused band or line 29 have not yet been exposed. Non-printed areas 34 are unexpanded.

In this exposure step, ink on the makeready sheet absorbs radiant energy, becomes heated, and in turn heats areas of the selectively-thermoexpansible layer of resinous material and puffing agent adjacent thereto by conduction. These areas soften, the puffing agent in the sheet is activated in the soft areas under conditions of heat, and the gas of the puffing agent produces bubbles in the softened areas causing them to swell. The thermoexpanded areas are then allowed to cool and generated gas remains entrapped in the expanded areas of the layer. Local areas of the printed sheet which have a high ratio of inked surface, i. e., solid or black tone areas, absorb a greater amount of radiant energy and cause a greater amount of gas formation by the puffing agent than areas where this ratio is small, e. g., middletone areas. Areas of the sheet not printed, i. e., highlight areas, do not absorb radiant energy or do so only to a slight extent insufficient to effect expansion thereof. The resulting sheet after exposure has a thickness relief corresponding to the tone of the printing form, being thickest in solid tone areas (and of greatest thickness in the center of such areas), thinnest

in non-printing or highlight areas, and of essentially graduated thickness between these extremes.

Conditions of radiant energy exposure are especially detailed in the disclosure set forth in connection with Example 1. It will be noted that exposure to intense radiation is brief to prevent charring of the selectively-thermoexpansible layer, and that intense and uniform radiation is necessary to achieve high and selective expansion of the heat-sensitive layer before any significant dissipation of heat has a chance to take place therethrough. While heat-sensitive, our expansible layers are poor conductors of heat.

After exposure, the sheet is returned to the impression cylinder and registered with the printing form, as for example by matching the punched holes in the underlying packing and the makeready sheet. In an ideal overlay construction, the makeready sheet is placed beneath two or three layers of heavy packing paper (each layer being approximately 0.006" thick). The sheet preferably is not buried too deeply in the packing on the impression cylinder inasmuch as the tendency is then to upset desired registration. The outermost layer on an impression cylinder ready for printing suitably may be a printing blanket or the like, as is well known in the art. However, the makeready sheet itself may be used as the outer layer, if desired.

In Figure 4 a makeready sheet hereof 22 is illustrated in registered position beneath one layer (chosen for clarity of illustration) of packing 24a upon impression cylinder 23. A layer of packing 24b is positioned beneath the makeready sheet. Selectively expanded areas 30, 31 and 32 of sheet 22 coat during printing with solid tone area 35 and middletone areas 36 and 37, respectively, of printing form 25, mounted on a suitable support 26. A paper sheet 38 is illustrated receiving the inked image of the printing form.

Our complete overlay makeready process may be accomplished in as short a period as 10 minutes as compared to prior art processes requiring, in many cases, an hour or more. One of the largest expense factors about makeready, i. e., printing delays or press down-time, is therefore greatly reduced.

If desired, overlay-type sheet materials processed according to the foregoing may be registered for underlay or interlay makeready constructions. In such constructions, the carrier web side of the sheet is positioned next to the underside of the printing form (or the mounting block), and the selectively expanded layer lowermost.

The following examples are illustrative but non-limitative of our invention. For convenient reference, the various characteristics of the sheet materials of Examples 1 through 7 are tabulated below in Table I. All of the sheet materials of Examples 1 through 7 were processed using our overlay makeready process and placed in registration beneath two layers of 6 mil (0.006") packing on an impression cylinder. Printing done on commercial apparatus with such makeready constructions gave prints of exceptionally fine quality. Solid tones were dense, highlights clean and middletones delicately shaded according to the density of printing elements, as desired.

#### EXAMPLE 1

|                            | Parts by weight |
|----------------------------|-----------------|
| Cellulose acetate butyrate | 90              |
| 5 Polyvinyl acetate        | 90              |
| Plasticizer                | 39              |
| Solvent                    | 500             |
| Paste                      | 12.8            |

The cellulose acetate butyrate was obtained under the trade name "½ Second Butyrate," which is a low viscosity but hard cellulose-derivative thermoplastic resin, having a melting range of approximately 284-338° F., an intrinsic viscosity in acetone at 25° C. of approximately 0.66 to 0.86, a molecular weight of approximately 30,000, an

acetyl content between approximately 12 to 15%, a butyryl content of 35 to 39%, a hydroxyl content of 0.5 to 1.2%, a free acidity content of approximately 0.03 maximum, and a maximum moisture content of approximately 3%.

The polyvinyl acetate was "Vinylite AYAT," which has an approximate softening point of 187° F., an intrinsic viscosity in cyclohexanone at 20° C. of 0.69, and a specific gravity of 1.18.

The plasticizer was "Paraplex G-20," which is a 100% sebacic acid ester type polymeric plasticizer containing no modifying oil. The solvent was a mixture of 40 parts toluene, 9 parts ethanol, and 1 part normal butanol.

The paste was made by milling the following constituents on a paint mill into a uniform blend:

|               | Parts |
|---------------|-------|
| Puffing agent | 2     |
| Plasticizer   | 2     |
| Solvent       | 1     |

The puffing agent, "Celogen," was p,p'-oxy bis (benzene sulfonyl hydrazide), which decomposes at raised temperatures beginning at approximately 266° F., releasing nitrogen gas. The plasticizer and solvent in the paste were the same as those constituents in the resinous mass of this example.

The components above, other than the paste, were stirred together until a smooth solution was obtained. To this solution was then added the paste and stirring continued until a uniform blend resulted. About 17 additional parts of solvent were then added to the mass to reduce its viscosity and the blend then coated on 42 pound "Minniform" paper (a bleached Kraft converting paper) marketed by the Minnesota and Ontario Paper Company. A wet coating thickness of approximately 20 mils (0.02") was employed. Some impregnation of the paper backing resulted. The coating was dried for approximately one-half hour at room temperature and then for approximately ten minutes at 160° F. and finally for approximately twenty minutes at 225° F. The steps employed to accomplish drying were for the purpose of removing as completely as possible all solvent and moisture from the coating. In addition the short heat conditioning treatment of approximately twenty minutes at 225° F. served to smooth and densify the coating and thereby impart increased moisture resistivity to the sheet.

The resulting sheet was inked with the pattern of a printing form using conventional oil base carbon pigment printers ink. The ink wet the smooth resinous surface uniformly and remained effectively distributed in the pattern of the face of the printing form employed. The inked sheet was then briefly subjected to uniform and intense radiant energy.

The source of radiation employed was a tungsten line-filament lamp mounted lineally in a sealed quartz tube; however, equivalent sources may be used. At 230 volts the lamp had a capacity of 650 watts. The tube was mounted along the axis of the internal focus of an elliptical reflector having a focal distance of 0.852 inch. The other focal axis of the reflector was in the open, i. e., outside the boundaries of the reflector. The inked makeready sheet was rapidly passed in front of the reflector in the plane of the external focal axis, with the concentrated line of radiation thereby being focused on a narrow strip of the printed surface. The width of the line concentration of focused rays was approximately three-sixteenths of an inch.

The temperature of the radiation source, as measured by an optical pyrometer, was 2460° Kelvin at an input of 300 volts giving 970 volt-amperes. Under these conditions the makeready sheet, resting on an insulating blanket, was passed twice below the light source at a speed of 80" per minute. Had the sheet been passed beneath this source at a speed of approximately 20" per minute, charring of the sheet would have resulted.

In solid tone areas the sheet expanded to a total thickness of approximately 10.7 mils, 3.2 mils above areas of the sheet not expanded. Other areas, such as middle-tone areas and highlight areas, expanded to a degree commensurate with the darkness of their tone, non-printing areas remaining unexpanded. For example, in a middletone area of 20% printing elements (80% non-printing or clear) the sheet expanded to approximately 8.1 mils, 0.6 mil above non-expanded areas. The processed sheet, in other words, presented a thickness relief corresponding to the tone of the printing form.

If a source intensity of radiation, i. e., infrared or equivalent, is too low during processing, insufficient expansion of the sheet results, or the sheet expands in a generally non-selective fashion. If a source intensity of radiation is too high, the makeready sheet hereof chars and loses its value as a corrective sheet in printing. For example, at a source temperature of 2310° Kelvin at 250 volts giving 720 volt-amperes, the printed sheet of this example was passed three times through the line focus of radiation at 60 inches per minute. The resulting selectively expanded sheet was barely suitable for use in printing. Its pattern of expansion was not as accurate in relief as that pattern exhibited by the sheet expanded according to the preferred conditions of radiation hereinbefore set forth. At a filament temperature of 2700° K. at 375 volts giving 1350 volt-amperes, the sheet of this example was passed three times at a speed of 110 inches per minute through the line focus of irradiated rays. Despite the rate at which the sheet was processed, expanded areas were charred. While solid tone areas of this sheet were expanded to approximately 4.5 mils above the surface of the sheet, they were charred and could not withstand any great printing pressures.

The sheet materials of Examples 2, 3 and 4 were processed using the preferred conditions of exposure set forth in this example.

#### EXAMPLE 2

|                                                       | Parts by weight |
|-------------------------------------------------------|-----------------|
| Cellulose acetate butyrate of Example 1               | 30              |
| Polyvinyl acetate of Example 1                        | 30              |
| Plasticizer of Example 1                              | 12              |
| Diethylenetriamine (curing agent for the epoxy resin) | 1.6             |
| Epoxy thermosetting resin                             | 12              |
| Puffing agent of Example 1                            | 2.1             |
| Solvent                                               | 165             |

The thermosetting resin employed was an epoxy condensation polymer of epichlorohydrin and bisphenol A commercially available under the designation "BR-18774," which consists of 100% solids having an epoxy equivalency of 180-210, and a viscosity at 25° C. of 10,000 to 15,000 cps. The solvent was a mixture of 40 parts toluene, 9 parts isopropyl alcohol and 1 part normal butyl alcohol.

The ingredients above were added to the solvent in the order listed and stirred until a uniform blend resulted. The blend was then knife-coated with an orifice of 0.025 inch upon 42 pound Minniform paper. The coating was air-dried at room temperature for approximately one-half hour, oven-dried for approximately 20 minutes at 150° F. and then 20 minutes at 225° F. The raised temperature of drying advantageously served to condition the resinous coating so that it became less moisture sensitive and to effect curing of the thermosetting resin.

We have employed a wide variety of puffing agents in makeready sheets such as set forth in the example. An intimate mixture of urea and biuret, which decomposes at approximately 300° F. releasing ammonia, has been employed. Potassium bisulfite has been employed. Even small quantities, e. g., on the order of 3% by weight, of ammonium aluminum alum, which releases its water of hydration at approximately 248° F., have been employed,

7  
EXAMPLE 3

|                            | Parts by weight |
|----------------------------|-----------------|
| Polyvinyl butyral          | 100             |
| Plasticizer of Example 1   | 20              |
| Toluene                    | 180             |
| Isopropyl alcohol          | 120             |
| Puffing agent of Example 1 | 6               |

The polyvinyl butyral employed here was obtained under the designation "Butvar B76," which is produced by hydrolyzing polyvinyl acetate to polyvinyl alcohol and reacting the alcohol with butyraldehyde to give polyvinyl butyral. It has a softening point of 170° F., a hydroxyl content of approximately 13.0% (calculated as polyvinyl alcohol) and a polyvinyl acetate content of approximately 2.5%.

The above ingredients were mixed together until a uniform blend resulted. This uniform blend was coated on 42 pound Minniform paper in a manner as set forth in Example 2, the coating dried to a tack-free consistency at room temperature, and then oven dried for approximately 20 minutes at 150° F. and 20 minutes at 225° F.

## EXAMPLE 4

|                            | Parts by weight |
|----------------------------|-----------------|
| Hard polystyrene resin     | 35              |
| Toluene                    | 65              |
| Puffing agent of Example 1 | 1               |

The hard polystyrene resin employed in this example was an unmodified polystyrene sold under the trade name "Styron 666." According to tests of the American Society for Testing Materials, it had a tensile strength of 6,000 to 7,000 p. s. i. (ASTM D638-49T), an elongation of 1.5 to 2.0% (ASTM D638-49T), a flexural strength of between 12,000 to 15,000 p. s. i. (ASTM D790-49T), a heat distortion range of 168° to 175° F. (ASTM D648-45T), and a Rockwell hardness of M68-80 (ASTM D785-48T).

To the solvent, toluene, was added the polystyrene polymer in particle form and stirring continued until the polymer was uniformly dissolved therein. The puffing agent was crushed to a particle size of approximately 1 mil or less and dispersed, i. e., blended thoroughly in the solution by stirring. A Waring blender may suitably be employed.

The resulting blend was coated, using an orifice 0.020" thick, upon .90 lb. fourdrinier paper commercially available under the trade name "Sanfast." A heavy backing is necessarily used with the expandable resin-layer of this example inasmuch as the non-plasticized resin layer of this example exhibits a relatively high tendency to cause curling when coated upon relatively thin light weight backings. After being applied to the heavy backing, the resin coat was air-dried for approximately one-half hour at room temperature and then oven-dried for 20 minutes at 150° F., followed by 20 minutes at 225° F.

## EXAMPLE 5

|                                        | Gram parts by weight |
|----------------------------------------|----------------------|
| Vinyl chloride-vinyl acetate copolymer | 1200                 |
| Plasticizer                            | 480                  |
| Amyl acetate                           | 624                  |
| Volatile petroleum naphtha             | 680                  |
| Puffing agent of Example 1             | 30                   |

The vinyl chloride-vinyl acetate copolymer was an organosol grade containing approximately 90 parts vinyl chloride to 10 parts vinyl acetate. It had an intrinsic viscosity in cyclohexanone at 20° C. of 1.20, and a fusion temperature of 250-300° F.

The plasticizer for the copolymer was a polymeric polyester type, available under the name "Paraplex G-60," believed to consist largely of epoxidized soybean oil. It had an average molecular weight of 1000, a specific gravity of 0.990, and a saponification number of 180

mgm. of KOH/gm. The naphtha used has a specific gravity (60° F./60° F.) of 0.733 to 0.735.

All ingredients above except the puffing agent were added to a 2-gallon jar half filled with porcelain balls of approximately one-half inch diameter. The jar was rolled for about 16 hours to thoroughly mill the contents, after which the puffing agent was added and milling continued for an additional 2½ hours. Milling time and conditions may vary depending upon the type of container employed, the size of hard balls used, etc.

The organosol mixture thus prepared was knife coated at a thickness of 20 mils upon a 3-mil thick brass foil, the surface of which had previously been roughened with sandpaper. The coating was dried for 2 minutes at 180° F. and fused for 5 minutes at 260° F., a temperature below the decomposition temperature of the puffing agent.

The resulting sheet was printed and heated to approximately 180° F. as measured by a surface pyrometer at the metal surface. The heated sheet was then exposed to radiant energy using conditions of actual exposure slightly less severe than those set forth in Example 1, resulting in the formation of a high graduated relief pattern in the resinous layer. Preliminary heating of a heat-conductive metal-backed sheet to an ambient temperature above approximately 150° F. but below the decomposition point of the puffing agent incorporated therein is believed to reduce lateral dissipation or transfer of heat in the backing during exposure to radiant energy, whereby erratic or poor expansion of the resinous layer of the sheet is avoided.

## EXAMPLE 6

A flexible non-woven fabric support 4 mils thick, formed by fusing randomly oriented fibers consisting of approximately 40% non-thermoplastic viscose (regenerated cellulose) fibers and approximately 60% thermoplastic cellulose acetate fibers, was impregnated with the organosol resin dispersion of Example 5 using a 3 mil orifice. This impregnating coating was air-dried for a few minutes at room temperature, and a second coating knifed thereover using a 20 mil orifice. The structure was then dried for 24 hours at room temperature.

The resinous layer of this sheet contained tiny discrete particles coherently held together. They could be crumbled from the sheet by rubbing the structure briskly, but under actual conditions in printing, did not flake, split, crack or become displaced. Using conditions of exposure to radiant energy set forth in Example 1, printed areas of the particulate layer, i. e., those inked areas absorptive of radiant energy, selectively fused into a tough, continuous phase. Highlight areas or non-inked areas not absorptive of radiant energy remained in an unfused state. Decomposition of the puffing agent took place at a point slightly above the point at which the particulate resinous layer fused; therefore, generated gas remained entrapped within the layer giving the desired graduated relief pattern.

Porous fabric backing members may be impregnated with any suitable material prior to coating. Makeready sheets having highly porous support members impregnated as well as coated with our resinous masses may be inked upon either side and exposed to radiant energy to form an appropriate relief for makeready.

## EXAMPLE 7

|                                                     | Gram parts by weight |
|-----------------------------------------------------|----------------------|
| Vinyl chloride-vinyl acetate copolymer of Example 5 | 50                   |
| Epoxy resin of Example 2                            | 15                   |
| Adipyl dihydrazide                                  | 0.5                  |
| Amyl acetate                                        | 63                   |
| Naphtha of Example 5                                | 30                   |
| Puffing agent                                       | 1.5                  |

Adipyl dihydrazide has a melting point of about 350° F., and at raised temperatures, i. e., temperatures near its

melting point, is a highly effective curing agent for epoxy resins. It is inert in this resinous mixture at room temperatures. Instead of adipyl dihydrazide, 2,4-toluene disulfonamide, malonyl dihydrazide, or other heat-activatable curing agents for epoxy resins may be employed. Malonyl dihydrazide acts not only as a curing agent for epoxy resins but also as a puffing agent.

The puffing agent used here, available under the name "Celenogen AZ," releases nitrogen gas on heat decomposition starting at about 385° F.

The ingredients above were milled together using the method of compounding set forth for Example 5, and knife-coated upon a backing of the type used for Example 1 with a 17 mil orifice. The coating was dried for about 6 minutes at room temperature and fused at 275° F. for three minutes. The uncured epoxy resin in the coating served to plasticize the vinyl resin.

This makeready sheet was processed using conditions of exposure only slightly less severe than those employed for the sheet of Example 1. During processing, the heat generated in selected areas absorptive of radiant energy was sufficient to partially cure those areas of the sheet, thereby enhancing their expanded strength. Other areas not absorptive of radiant energy, and not therefore heated, remained uncured. If desired the epoxy resin in such areas may be cured by a short heating step just below the temperature of decomposition of the puffing agent.

In the following table various characteristics, as identified, of the foregoing makeready sheets are tabulated.

Table I

| Example | 1    | 2    | 3    | 4    | 5    | 6    | 7    |
|---------|------|------|------|------|------|------|------|
| a       | 3.5  | 3.5  | 3.5  | 7.0  | 3.0  | 4.0  | 3.5  |
| b       | 7.5  | 8.5  | 8.0  | 14.0 | 9.0  | 9.0  | 7.3  |
| c       | 4.0  | 5.0  | 4.5  | 7.0  | 6.0  | 5.0  | 3.8  |
| d       | 10.7 | 13.5 | 11.5 | 17.5 | 13.5 | 17.0 | 11.3 |
| e       | 3.2  | 5.0  | 3.5  | 3.5  | 4.5  | 8.0  | 4.0  |
| f       | 9.5  | 11.5 | 10.0 | 17.0 | 11.8 | 13.0 | 11.1 |
| g       | 2.0  | 3.0  | 2.0  | 3.0  | 2.8  | 4.0  | 3.8  |
| h       | 0.9  | 0.9  | 0.8  | <0.5 | <0.5 | <0.5 | <0.5 |
| i       | 2.8  | 2.8  | 2.4  | <0.5 | 0.9  | 0.9  | <0.5 |

a. Thickness of backing in mils (thousandths of an inch).

b. Total mil thickness of unexpanded dry sheet material.

c. Thickness of selectively thermoexpansive layer (b-a).

d. Total thickness of sheet material in maximally expanded areas, i. e., solid tone areas, measured at room temperature after processing according to the teachings herein.

e. Differential in thickness between maximally expanded areas and the initial thickness of the sheet or unexpanded areas (d-b).

f. Total mil thickness of processed sheet material in maximally expanded areas under a pressure of 250 p. s. i. for 15 seconds at room temperature.

g. Differential in thickness of processed sheet material between maximally expanded areas under a pressure of 250 p. s. i. for 15 seconds at room temperature and the initial thickness of the sheet or unexpanded areas (f-b).

h. Weight percent of dissolved water in the unexpanded selectively thermoexpansive layer after conditioning for three days at 56% R. H. and 75° F.

i. Weight percent of dissolved water in the unexpanded selectively thermoexpansive layer after conditioning for three days at 93% R. H. and 80° F.

In the foregoing examples we used solution or dispersion coating methods to fabricate our sheets; however, other methods such as calendering, extruding, etc., may be used. The important requirement is that the resulting coat must be at least about 2 mils thick over the entire backing member or carrier web and should be of essentially uniform thickness. Any suitable method may be used to accomplish this result.

Small amounts of various inert fillers and materials, for example, aluminum powder, calcene, silica fines, bentonites, etc., may be incorporated in a uniformly dispersed condition in the resinous layers of our sheets.

Our sheet materials may be characterized as essentially of uniform thickness and as flat-lying in that they remain substantially flat and resist curling, warping, etc., during processing. Overlay-type sheets such as those of the foregoing examples are preferably not more than

about 12 mils thick for the reason that more accurate control of the desired packing and of registration on an impression cylinder is possible with such sheets.

The carrier web is dimensionally-stable or planarly-stable in that it imparts planar stability, i. e., resistance to curling, warping, stretching, etc., to the makeready sheet. Registration of the sheet material after processing is thereby easily accomplished. In the most ideal sheet structures, the backing member is between approximately 2 and 5 mils in thickness. Other flexible backings than those set forth in the examples may be employed. For example, non-fibrous films of glycol-terephthalate polymer ("Mylar"), cellulose acetate, silk screens, various metal sheets or foils, various laminates of materials, impregnated materials, etc. are employable. At least one surface of the backing material is preferably of a sufficiently fibrous nature for anchorage of the selectively-thermoexpansive resinous layer thereto; however, smooth surfaced backing sheets may be roughened to secure adhesion or bonding of the resinous layer thereto, as illustrated in Example 5, or an interposing layer of adhesive may be used to firmly bond the backing and resinous layer together.

Preferred overlay-type sheets hereof have backing members characterized as of low heat conductivity, particularly if compared to the conductivity of metals, so that lateral diffusibility of heat through the backing support from limited localities thereof affected by heat in adjacent portions of the adhered resinous layer during processing is minimized. We may, however, as in Example 5, employ thin flexible heat-conductive metal backing members. Metal backings inherently possess desirable properties of strength and dimensional stability.

Backings are preferably light in color for the reason that many dark colored backings coated with translucent layers absorb infrared rays. We realize, however, that dark colored backings may be used and a highly reflective or opaque resinous coating employed or a different range of radiant energy employed, to selectively expand the sheet according to selective absorption by a special ink having absorptive powers for the particular rays employed. This we consider an equivalent of our invention.

Likewise, although in the preferred embodiment our sheets are printed with inks having high absorptivity for infrared rays, e. g., black ink, we may employ other inks having absorptive qualities for a different range of radiation than infrared rays and use resinous layers and backings which do not absorb these rays, or which do so only to a slight extent. This, also we consider an equivalent.

The resinous material in our selectively thermoexpansive layer is usually polymeric and must be thermosoftenable as may be noted from the examples and illustrations hereof. Preferably, at least one hard hydrophobic thermoplastic polymeric material is employed in making up the layer. Materials having a Shore D Durometer hardness above 40 are generally preferred, but such a hardness value is somewhat misleading inasmuch as softer materials which are thermosetting or curable to suitable hardness in processing may be used. Resins which are thermosetting but temporarily thermoplastic, which are thermoplastic and vulcanizable, as well as others and in various combinations—all are employable if in the final coat after heat softening, puffing and cooling, the selectively expanded resinous layer is non-brittle (particularly as compared to abietic acid or rosin) and possesses sufficient hardness, resilient strength and toughness to resist flattening in use, e. g., to maintain approximately a 2 mil differential in thickness between (a) fully or maximally expanded areas after 15 seconds under a pressure at least as high as approximately 250 p. s. i. (lbs./in.<sup>2</sup>), and (b) those areas of the sheet not expanded. Such conditions of time and pressure are

believed to closely approximate those encountered under most actual printing conditions.

Also employable together in the layer are resins and other components which are incompatible, but which after drying, do not sublime or migrate from the layer. A coating of non-compatible resins and other components may be heated slightly to improve the dry stability thereof. Preferred selectively thermoexpansive layers have a uniform smooth fused appearance, but, as illustrated in Example 6, our layers may be comprised of a plurality of individual particles.

Preferably the dry thickness of the selectively thermoexpansive layer in makeready sheets especially designed for overlay use is between approximately 2 and 7 mils but may be as great as 12 mils, or greater, with satisfactory results. By dry we mean normally less than about 3% volatile organic solvent by weight, so as to prevent blocking of stacked sheets and so as to avoid unnecessary weaknesses in the layer upon expansion. A thickness of at least 2 mils is needed if high graduated relief patterns are to be formed. Thinner coats fail to expand reliably and even lose gas generated therein. Our layers generally contain small amounts of organic, usually polymeric, plasticizers for their thermoplastic resinous components because of the advantageous planar stability, i. e., reduction of tendency to curl and warp, as well as in some cases increased moisture resistance, imparted to the resulting layer. Plasticizers, however, almost invariably somewhat reduce expanded strength of a resinous layer. Accordingly, the layer of such sheets is generally at least about 3 mils thick, and usually between 4 and 7 mils thick for best results in terms of maintaining suitable expanded thickness differentials under pressure. Layers greater than approximately 12 mils thick are generally undesirable because expanded areas are apt to be displaceable under compression, and desired high differentials in thickness are apt to be reduced because of the greater relative compressibility of such thick coats. This disadvantage of thick coats or layers may be corrected to some extent by incorporating therein suitable curing agents or thermosetting resins.

The dispersed, heat-sensitive, normally-dormant, puffing agent in the selectively-thermoexpansive layer remains therein in a storable, stable condition. It may, in fact, react with the resinous mass, cure it, or even be a molecular component of a resin, so long as it retains its required ability to expand the layer under conditions of heat. Finely pulverized, uniformly dispersed, particles of a puffing agent facilitate the formation of a large number of tiny bubbles or cavities in the resinous layer, with a great number of connecting columns of resin, all of which contributes to the strength and resiliency of expanded areas, as well as to the formation of well-regulated graduated relief patterns.

The amount of puffing agent employed may vary depending upon the relative ability of the agent to expand the sheet under conditions of heat employed in processing. A resinous layer may contain as little as approximately 1% by weight of a highly efficient puffing agent, e. g. "Celogen," but may require up to approximately 30% by weight of a less efficient agent. Amounts in excess of approximately 10% by weight are generally to be avoided inasmuch as certain weaknesses are apt to develop within the sheet. However, an inefficient puffing agent which contributes to the strength of the sheet may be suitable to employ in high concentrations. Preferred puffing agents chemically decompose at raised temperatures to give off a gas; however, materials or puffing agents which act by vaporization on heating, as opposed to decomposition, while inferior, may be suitable to use.

The preferred temperature range at which expansion of our heat-sensitive makeready sheets occurs is well above room temperature and is between approximately 150° F. and 350° F., but may be as high as 450° F., or even considerably higher. Expansion at exceedingly

low temperatures is generally unreliable and not controllable; on the other hand, expansion which does not occur until exceedingly high temperatures, i. e., those for example over about 450 or 500° F., are attained creates problems with respect to suitable exposure conditions for processing as well as with respect to obtaining suitable graduated relief patterns.

The temperature at which our resinous masses soften and the temperature at which a puffing agent incorporated therein gives off gas should generally be within approximately the range of 75° F. of each other, although for some less critical combinations, a temperature difference as great as about 150° F., or even greater, has been found useful. Generally, however, it has been found that if a puffing agent generates gas at a temperature too far below that at which a resinous layer softens, control of expansion becomes difficult and desired graduated relief patterns are not easily obtained. If, on the other hand, the puffing agent releases gas only at temperatures greatly above those at which the resinous material softens, difficulty arises with respect to maintaining the released gas within the softened resinous layer so as to expand the same. The faults of extremes are easily avoided if materials are selected with a view toward maintaining the activation temperature for the puffing agent reasonably close to the softening temperature of the resinous layer.

The selectively-thermoexpansive layer of our sheets has a prolonged shelf life and may be characterized as hydrophobic in that it resists imbibition of water or moisture to an extent that it does not contain sufficient dissolved water, even after being stored under atmospheric conditions, to interfere greatly with the gaining of high, graduated, tough and sturdy relief patterns when it is later exposed to radiant energy during processing as taught herein. The foregoing definition for the required hydrophobic nature of our heat-expansive layers is far more accurate than quantitative figures on their maximum permissible moisture content; although, when using such a standard, the heat-expansive layer of our sheets does not contain, even when exposed for lengthy periods to especially adverse conditions of temperature and moisture, more dissolved water than from 0 up to 4% by weight. Expansible layers which contain more than about 4% water by weight give unreliable results in expansion and erratic relief patterns, frequently of greater thickness in middletone than solid tone areas, when made heat-sensitive and processed as taught herein. In Table I qualitative data as to the dissolved moisture content in the selectively-thermoexpansive layers of the foregoing examples is set forth. Particular note should be taken of those low values obtained when the articles of the examples were stored under high humidity conditions such as might be encountered in summer months.

The surface of our selectively expandable layers may be characterized as lyophilic or organophilic in that it accepts conventional printing inks readily and is not deleteriously affected thereby, even though the printing inks contain oils and the like. The ink receptive nature of our selectively expandable layers may be appreciated when it is realized that areas inked upon our sheets are not significantly altered in shape by such phenomenon as surface tension which may cause an inked area to pull-up into globules. Instead the ink wets the resin surface and remains in position upon the sheet substantially as it was originally applied.

Our sheets after processing do not flake, split, crack, become pulverized, or exhibit cold flow under conditions of use. We believe that the selective and proportionate resiliency, toughness, and strength of our selectively expanded layers, including their ability to resist crushing and displacement as well as flattening compressive forces such as are encountered in printing, i. e., "press pounding," accounts in a large measure for the especially fine

printing results obtained when our sheets are employed as taught herein.

According to another embodiment of this invention, there is provided a novel process and also makeready sheet materials for "bumping-up" or distorting electrotypes, photoengravings and the like in a very accurate manner for appropriate impression pressure corrections in printing. In a "bump-up" plate treatment process, a positive paper cutout relief sheet with dark tones raised is registered under a printing form, e. g., an electrotype, and a negative paper cutout, i. e., one with highlight tones raised in relief, is registered over the electrotype. This laminate is then placed between rigid metal plates and the resulting laminate passed between squeeze rollers, which action deforms the electrotype, raising dark tones relatively to highlights. The so distorted electrotype is shaved smooth on its back surface before the negative sheet is removed, and thereafter, is mounted on a suitable base for printing.

Example 8 illustrates this specialized embodiment of our invention. As will be evident, the general characteristics of overlay sheets above set forth are also applicable to sheets of this embodiment of our invention. The sheets of this embodiment, however, possess a greater strength in expanded areas.

#### EXAMPLE 8

|                                                                                    | Parts by weight |
|------------------------------------------------------------------------------------|-----------------|
| Epoxy thermosetting resin of Example 2                                             | 60              |
| 2,4-toluene disulfonamide (Epoxy curing agent)                                     | 8               |
| N-(3 diethylaminopropyl) phthalimide salicylate (Activator for epoxy curing agent) | 0.7             |
| Vinyl chloride-vinyl acetate copolymer of Example 5                                | 80              |
| Amyl acetate                                                                       | 80              |
| Naphtha of Example 5                                                               | 60              |
| p-Diphenyldiazonium fluoborate (puffing agent)                                     | 4               |

For the positive sheet, the above ingredients were milled together to form a uniform dispersion by following the method of compounding set forth in Example 5.

For the negative sheet, the same ingredients, quantities and process were used except that 2 parts by weight of activated carbon black ("Carbolac #2") were added to the mixture about 1½ hours before milling was terminated. Instead of using a pigment absorptive of radiant energy, we may use a radiation-absorbent backing or carrier web with a transparent coating and thereby attain an equivalent sheet.

Each dispersion was then knife-coated on a separate carrier web of the type used in Example 1 with 18 mil orifices. Other backings as discussed hereinbefore may be used. The coatings were dried 15 minutes at room temperature and 15 minutes at 150° F. The dried coatings remained in an unfused state; however, the vinyl chloride-vinyl acetate copolymer particles in the dried layer were swelled by what appeared to be a plasticizing action on the part of the uncured epoxy resin in the coating, and the swelled resin particles seemed to be bonded to each other by the epoxy constituent in the layer. The dried sheet was about 8.5 mils thick, 3.5 mils of which was backing.

The dry positive sheet was inked with an impression of the electrotype to be bumped. Black ink pigmented with carbon-black was employed. The negative sheet was inked also with an impression of the electrotype but in this case a radiation reflecting or non-absorbing ink was used. Silver ink having a reflective silver or aluminum pigment is satisfactory. Each sheet was then exposed to brief, intense and uniform radiation. Suitably, conditions only slightly less severe than those described in Example 1 are employed. The processed sheets of this example in maximum expanded areas were 14.5 mils thick, 3.5 mils of which was backing, and these areas supported pressures of about 100 p. s. i. for 15 seconds remaining at least about 5 mils above areas not expanded. No oven curing was necessary to achieve such strength

in the selectively expanded layers of this example, but an oven curing step may be used if desired.

The p-diphenyldiazonium fluoborate functioned during exposure of this sheet not only as a puffing agent but also as a curing agent for the epoxy resin in those selected areas heated. Other such agents are p-aminodiphenyldiazonium fluoborate, p-toluene diazonium fluoborate, etc.

Referring now to Figure 5 for illustration, the positive sheet 39, inked with radiant energy absorptive ink 40 and 41, increased in thickness in those areas, the greatest increase taking place in solid tone area 40. The negative sheet 42, inked with radiant energy reflective ink 43 and 44, increased in thickness in non-inked areas 45 and 46, and exhibited the greatest increase in area 45 on which no reflective ink was printed. The hard and tough cured sheets were each in relief form; however, the relief of the negative sheet 42 was the reverse of that of the positive sheet 39. The positive sheet 39 was then registered 20 underneath the electrotype 47, and the negative sheet 42 registered above the electrotype. This laminate was then placed between rigid metal plates 53 and 54 and the resulting laminate passed between squeeze rollers 48 and 49. By this process, the electrotype was distorted, i. e., 25 bumped, in extremely accurate detail. Solid tone area 50 was raised relatively to highlight areas 51. Likewise middle tone area 52 was raised relatively to highlight areas 51 but was not raised to the same relative degree that the solid tone area was raised. The electrotype was, 30 in other words, given a relief distortion. The positive sheet was then removed, the back of the electrotype was leveled, i. e., shaved smooth, and the negative sheet removed. Prints made using this treated electrotype in suitable well-known printing arrangement were of the 35 exceptionally fine quality aforescored.

The resistance to moisture imbibition of the sheet materials of this example is as follows: In a test for 3 days at 56% R. H. and 75° F., as well as in a test for 3 days at 93% R. H. and 80° F., the selectively thermoexpansive 40 layers in each case contained less than 0.5% by weight dissolved water.

Great strength is required in the expanded portions of these positive and negative sheets. The strength of the expanded areas, usually cured, is sufficient to support at 45 least 1,000 p. s. i. for 15 seconds and still remain at least more than 2 mils and generally at least approximately 5 mils above the unexpanded portions of the sheet. These sheets therefore, are the more unusual when it is realized that such strength is gained in vesicular expanded portions. While these sheets may also be used as overlay-type makeready sheets, they frequently possess more than 50 the desired strength for usual overlay makeready requirements.

Our negative sheets, i. e., sheets hereof which are absorptive of radiant energy and are processed using reflective inks to mask out areas not to be expanded, may be used also in a "bump-up" process without the positive sheet, if desired. In such a process, the negative sheet is printed with the pattern of the electrotype using a reflective ink, and thereafter, it is exposed to radiation, as herein taught, and registered over the electrotype. Next, pressure is applied over all points or areas of the back surface of the electrotype to distort it toward and according to the relief of the negative sheet. The back 60 surface of the "bumped up" electrotype is then shaved smooth and the resulting corrected electrotype is ready for printing.

In another embodiment of our invention, both sides of a carrier web are coated with a selectively-thermoexpansive layer. To selectively expand both sides of such a sheet, the following procedure may be followed: A smooth outer cover, preferably with a hard glazed surface, is first wrapped around an impression cylinder and printed upon. A double-coated makeready sheet 75 then is wrapped around the impression cylinder over the

aforementioned printed outer cover and the outside surface of the makeready sheet printed upon. During the second printing step, the mirror image of the printing form is printed by offset upon the side of the makeready sheet in contact with the originally printed glazed wrapping. Each side of the makeready sheet is then exposed to radiant energy to expand the same, and the expanded sheet placed in registration as desired.

A novel method for gaining registration of overlay makeready using relatively thin translucent sheets such as the one of Example 1 hereof, is as follows: A plain sheet of paper is wrapped around an impression cylinder, printed with an impression of a printing form, marked for subsequent registration, and removed from the cylinder. The translucent makeready sheet is then printed with an impression of the printing form, exposed to radiant energy, adhesively secured over the previously printed sheet of paper in registration with the print thereon, and the whole structure registered on the impression cylinder using the indicia markings on the plain sheet of paper.

For linotype printing, it is sometimes desired to increase the packing thickness over certain lines so as to obtain appropriate ink transfer to paper being printed. When using our makeready sheet material non-absorptive of radiant energy to accomplish this, one first marks or shades various selected areas of the sheet material with radiant energy absorptive ink or pencil according to the desiderata for increased thickness over various lines or areas of a linotype printing form. Suitably, markings or shadings of different infrared-absorptive qualities may be made by using various pencils, inks, crayons, etc., each with different infrared-absorptive qualities, or by applying black ink or the like in various shades or density over various lines or areas of our sheet material. The so-marked sheet is then exposed and expands selectively according to the infrared absorptivity of the marked areas. It is then registered appropriately so as to cooperate with a linotype form in printing.

Makeready sheets hereof may also be used in making novel "sandwich" printing form constructions. One such construction is that gained by registering a selectively expanded makeready sheet, e. g., a positive-type or overlay-type makeready sheet as above set forth, beneath an electrotype, or the like, and adhesively bonding the two together. The back side of the electrotype may be shaved down so that the electrotype itself is extremely thin. A thin sheet of metal of uniform thickness may be adhesively secured to the bottom side of the structure, i. e., beneath the selectively thermoexpanded layer of the registered makeready sheet, to contribute to the strength of the whole structure, if desired. Another "sandwich" type construction results if an electrotype, or the like, which suitably may be shaved thin, is pressed into a coating of a heat-hardenable, resinous adhesive on a uniform metal backing by using a negative type makeready sheet, as above described, in register over the electrotype. The negative sheet, selectively expanded in highlight areas, will deform the thin electrotype into the adhesive layer when pressure is applied thereover. The heat-hardenable resinous adhesive may substantially simultaneously be activated to hold the plate in deformed condition.

A selectively thermoexpansible layer, as well as the backing, for our makeready sheets may be formed from a wide variety of materials. Because new polymeric hydrophobic resinous materials and new puffing or blowing agents are continually being developed and marketed, it is impossible to catalogue all components useful in a heat-sensitive layer. Further such a catalogue by specific chemical names would be misleading in that our invention relating to sheet materials does not lie in any specific single chemical component but rather in the new and useful combination and structure having new and useful physical properties, as taught herein. For those wishing to use new materials which may become available, it will

be a simple expedient, after studying the foregoing, to make routine tests and to utilize available knowledge in the light of this specification to determine whether the new materials are suitable. Good judgment will necessarily be exercised but it is safe to assume that no one will wish to make and process a useless sheet material or will be misled by the foregoing into making and processing worthless articles using new materials and ingredients which may become available.

We are aware of prior art patents teaching sheet materials which are light-sensitive or photosensitive and are useful in making photographic-type images. These patents are unrelated to makeready for letterpress printing. In general, it may be noted that the sheet materials of these patents have thin hydrophilic, even water-soluble, layers which are not designed to give high, graduated, tough and sturdy relief patterns upon exposure to radiant energy as taught herein.

What is claimed is as follows:

- 20 1. A flexible, flat-lying, unitary sheet material of essentially uniform thickness adapted for makeready in letterpress printing by a process involving differential sustained expansion, said sheet material comprising a flexible, planarly-stable, carrier web, and, on at least one side thereof, a flexible, selectively-thermoexpansible, ink-receptive, hydrophobic layer comprising a hydrophobic, at least temporarily thermosoftenable, resinous material and, uniformly distributed therethrough, a normally-dormant, heat-sensitive, puffing agent activatable at a temperature well above normal room temperature to expand said layer under conditions of heat, said puffing agent being present in an amount sufficient to provide on rapid and complete heat-activation of said layer an increase of at least 2 mils in the thickness thereof, and said layer being hardenable in expanded condition to an extent sufficient to support pressures at least on the order of 250 p. s. i. for about 15 seconds while maintaining areas of maximum expansion at least approximately 2 mils greater than the initial thickness thereof.
- 25 2. The article of claim 1 in which the selectively-thermoexpansible layer contains a thermosetting resin.
- 30 3. The article of claim 2 in which the selectively-thermoexpansible layer contains a curing agent for said thermosetting resin.
- 35 4. The article of claim 1 in which the selectively-thermoexpansible layer is at least about 3 mils thick and contains an organic plasticizer.
- 40 5. The article of claim 1 in which the selectively-thermoexpansible layer contains a material absorptive of radiant energy.
- 45 6. A flexible, flat-lying unitary sheet material of essentially uniform thickness adapted for makeready in letterpress printing by a process involving differential sustained expansion, said sheet material comprising a flexible, planarly-stable, carrier web, and, on at least one side thereof, a flexible, selectively-thermoexpansible, ink-receptive, hydrophobic layer at least 2 mils thick and comprising a hydrophobic thermoplastic resin, a thermosetting resin and, uniformly distributed through said resins, a normally-dormant, heat-sensitive, puffing agent activatable at a temperature well above normal room temperature to expand said layer under conditions of heat, said puffing agent being present in an amount sufficient to provide on rapid and complete heat-activation of said layer an increase of at least 2 mils in the thickness thereof, and said layer being hardenable in expanded condition to an extent sufficient to support pressures at least on the order of 250 p. s. i. for 15 seconds while maintaining areas of maximum expansion at least approximately 2 mils above the initial thickness thereof.
- 50 7. The article of claim 6 in which the selectively-thermoexpansible layer contains a curing agent for the thermosetting resin.
- 55 8. A flexible, flat-lying, unitary sheet material of essentially uniform thickness adapted for makeready in

letterpress printing, said sheet material being characterized by an ability to expand in selected areas to present a relief according to a pattern inked thereon with ink highly absorptive of radiant energy, said sheet being sufficiently less absorptive of said radiant energy so that, upon exposure of said sheet after inking to brief, intense, and uniform radiant energy only those portions inked will expand commensurately with the amount of inking placed thereon to present a relief pattern thickest in solidly inked areas and thinnest in non-inked areas, and of graduated thickness in other areas approximately according to the density of ink thereon, said sheet comprising: a flexible, planarly-stable, carrier web of low heat conductivity, and a flexible, selectively-thermoexpansive, ink-receptive, hydrophobic layer on at least one side of said carrier web, said layer being at least 2 mils thick and comprising a hydrophobic thermoplastic resin, a thermosetting resin and, uniformly distributed through said resins, a normally-dormant, heat-sensitive, puffing agent activatable at a temperature well above normal room temperature to expand said layer under conditions of heat, said puffing agent being present in an amount sufficient to provide on rapid and complete heat-activation of said layer an increase of at least 2 mils in the thickness thereof, and said layer being hardenable in expanded condition to an extent sufficient to support pressures at least on the order of 250 p. s. i. for 15 seconds while maintaining areas of maximum expansion at least approximately 2 mils above the initial thickness thereof.

9. The article of claim 8 in which the selectively-thermoexpansive layer contains a curing agent for the thermosetting resin.

10. A flexible, flat-lying, unitary sheet material of essentially uniform thickness adapted for makeready in letterpress printing by a process involving differential sustained expansion, said sheet material comprising a flexible, planarly-stable, carrier web, and, on each side thereof, a flexible, selectively-thermoexpansive, ink-receptive, hydrophobic layer comprising a hydrophobic, at least temporarily thermosoftenable, resinous material and, uniformly distributed therethrough, a normally-dormant, heat-sensitive, puffing agent activatable at a temperature well above normal room temperature to expand said layer under conditions of heat.

11. In a process of makeready for letterpress printing, the step of briefly exposing a makeready sheet comprising a flexible, selectively-thermoexpansive layer, and having a differentially radiation-absorptive makeready pattern thereon, to uniform and intense radiant energy differentially absorptive by elements of said pattern to provide a heat pattern sufficient to expand said layer selectively.

12. In a process of makeready for letterpress printing, the step of briefly exposing a makeready sheet non-absorptive of radiant energy comprising a flexible, selectively-thermoexpansive layer, and have a makeready pattern thereon of radiant energy absorptive elements, to uniform and intense radiant energy sufficient to expand the layer in selected areas in heat-conductive association with the radiant energy absorptive elements.

13. In a process of makeready for letterpress printing, the step of briefly exposing a makeready sheet absorptive of radiant energy comprising a flexible, selectively-thermoexpansive layer, and having a makeready pattern thereon of radiant energy reflective elements, to uniform and intense radiant energy sufficient to expand said layer in selected areas absorptive of radiant energy.

14. A process of makeready for letterpress printing including the steps of inking a differentially radiation-absorptive pattern upon a makeready sheet comprising a flexible, ink-receptive, selectively-thermoexpansive layer, and briefly exposing said inked makeready sheet to uniform and intense radiant energy differentially absorptive by elements of said pattern to provide a heat pattern sufficient to expand said layer selectively.

15. A process of makeready for letterpress printing comprising (1) inking a differentially radiation-absorptive pattern upon a makeready sheet comprising a uniform, flexible carrier web of low heat conductivity, and, firmly bonded thereto, an ink-receptive, heat-sensitive, coating of uniform thickness comprising a thermosoftening, resinous material containing, uniformly distributed therethrough, a heat-sensitive, puffing agent, and (2) briefly exposing said inked sheet to uniform and intense radiant energy differentially absorptive by elements of said pattern to provide a heat pattern sufficient to selectively expand said sheet, said expanded sheet possessing sufficient strength and toughness in fully expanded areas to maintain at least a thickness variation of approximately 2 mils under a pressure at least as high as approximately 250 p. s. i.

16. A process of makeready for letterpress printing comprising (1) inking a pattern with a radiant energy absorptive ink upon a makeready sheet substantially non-absorptive of radiant energy and comprising a thermosoftenable resinous material having a heat-sensitive puffing agent uniformly distributed therein, and (2) briefly exposing the inked pattern of said makeready sheet to uniform and intense radiant energy sufficient to heat and expand said sheet in selected areas in heat conductive association with said radiant energy absorptive ink.

17. A process of makeready for letterpress printing comprising (1) inking a pattern with radiant energy reflective ink upon a makeready sheet absorptive of radiant energy and comprising a thermosoftenable resinous material having a heat-sensitive puffing agent uniformly distributed therein, and (2) briefly exposing the inked makeready sheet to uniform and intense radiant energy sufficient to heat and expand said sheet in selected areas absorptive of radiant energy.

18. A process of makeready for letterpress printing comprising (1) inking a makeready pattern upon a flexible, selectively-thermoexpansive layer of a makeready sheet to provide differential radiation absorptivity, said layer containing a resinous material and a puffing agent, (2) raising said inked makeready sheet to an ambient temperature above room temperature but below the activation temperature for said puffing agent, and then, (3) briefly exposing said inked layer to uniform and intense radiant energy differentially absorptive by elements of said pattern to provide a heat pattern sufficient to expand said layer selectively.

19. A process of makeready for letterpress printing comprising (1) placing a makeready pattern on a flexible, selectively-thermoexpansive layer containing a resinous material and a puffing agent to provide differential radiation absorptivity, (2) briefly exposing said layer to uniform and intense radiant energy to provide, according to said makeready pattern, a heat pattern sufficient to expand said layer selectively, and (3) registering said selectively expanded layer with a printing form.

20. A process of makeready for letterpress printing comprising (1) inking a printing form makeready pattern reflective of radiant energy upon a flexible, ink-receptive, selectively-thermoexpansive layer absorptive of radiant energy, said layer containing a resinous material, a material absorptive of radiant energy and a puffing agent, (2) briefly exposing said inked layer to uniform and intense radiant energy sufficient to heat and expand said layer in selected areas which absorb radiant energy, said layer being formed so as to be sufficiently hard and tough in selectively expanded areas to maintain maximally expanded areas at least 2 mils greater than the initial thickness thereof while under a pressure on the order of 1000 p. s. i. for about 15 seconds, (3) registering said selectively expanded layer over the printing surface of said printing form, and (4) applying pressure over areas of the back of said printing form so as to

distort it according to the relief of said registered selectively expanded makeready sheet.

21. A process of makeready for letterpress printing comprising (1) inking a pattern of a printing form with radiant energy absorptive ink upon a positive makeready sheet substantially non-absorptive of radiant energy and comprising an ink-receptive, selectively-thermoexpansible layer containing thermosoftening hardenable resinous materials and a puffing agent, (2) inking a pattern of the printing form with radiant energy reflective ink upon a negative makeready sheet of a construction such as described in step (1) but containing a radiant energy absorptive material in uniform heat-conductive association therewith, (3) briefly exposing each sheet to uniform and intense radiant energy sufficient to selectively expand the layers thereof in areas affected by heat generated from absorbed radiant energy, said selectively-expanded layers being formed so as to be sufficiently hard and tough to maintain maximally expanded areas at least 2 mils greater than the initial thickness thereof while under a pressure on the order of 1000 p. s. i. for about 15 seconds, (4) registering said selectively-expanded positive sheet below said printing form and said selectively-expanded negative sheet above said printing form, and (5) applying pressure over all areas of said laminate so as to distort said printing form by raising solid tone areas and depressing highlight areas.

22. A flexible, flat-lying, unitary sheet material of essentially uniform thickness adapted for makeready in letterpress printing by a process involving differential sustained expansion, said sheet material comprising a flexible, planarly-stable, carrier web, and, on at least one side thereof, a flexible, selectively-thermoexpansible, ink-receptive, hydrophobic layer at least 2 mils thick and comprising a hydrophobic, at least temporarily thermosoftenable, tough, resinous material and, uniformly distributed therethrough, a multitude of fine particles of a normally-dormant, heat-sensitive, puffing agent activatable at a temperature well above normal room temperature to produce a gas as a result of chemical decomposition and thereby expand said layer under conditions of heat, said puffing agent being present in an amount sufficient to provide on rapid and complete heat activation of said layer an increase of at least 2 mils in the thickness thereof, and said layer being hardenable in expanded condition to an extent to support pressures at least on the order of 250 p. s. i. for about 15 seconds while maintaining areas of maximum expansion at least approximately 2 mils greater than the initial thickness thereof.

23. A flexible, flat-lying, unitary sheet material of essentially uniform thickness adapted for makeready in letterpress printing by a process involving differential sustained expansion, said sheet material comprising a flexible, planarly-stable, carrier web, and, on at least one side thereof, a flexible, selectively-thermoexpansible, ink-receptive, hydrophobic, at least temporarily thermosoftenable layer at least 2 mils thick and comprising a hydrophobic thermoplastic resin, a thermosetting resin, a heat-activatable curing agent for said thermosetting resin, and, uniformly distributed through said layer, a multitude of fine particles of a normally-dormant, heat-sensitive, puffing agent activatable at a temperature well above normal room temperature to produce a gas as a result of chemi-

cal decomposition and thereby expand said layer under conditions of heat, said puffing agent being present in an amount sufficient to provide on rapid and complete heat activation of said layer an increase of at least 2 mils in the thickness thereof, and said layer being hardenable in expanded condition to an extent to support pressures at least on the order of 250 p. s. i. for about 15 seconds while maintaining areas of maximum expansion at least approximately 2 mils greater than the initial thickness thereof.

24. The sheet material of claim 23 wherein the heat-sensitive puffing agent is activated to produce a gas within approximately 150° F. of the thermosoftening temperature of the selectively-thermoexpansible layer.

25. The sheet material of claim 24 wherein the carrier web is of low heat conductivity.

26. The sheet material of claim 23 wherein the selectively-thermoexpansible layer contains a material which absorbs radiant energy, said sheet material being further characterized in that its layer is hardenable in expanded condition to an extent to support pressures at least on the order of 1000 p. s. i. for about 15 seconds while maintaining areas of maximum expansion at least approximately 2 mils greater than the initial thickness thereof.

27. A flexible, flat-lying, unitary sheet material of essentially uniform thickness adapted for makeready in letterpress printing by a process involving differential sustained expansion, said sheet material comprising a flexible, planarly-stable, carrier web at least about 2 mils thick and of low heat conductivity, and, on at least one side thereof, a flexible, selectively-thermoexpansible, ink-receptive, hydrophobic, at least temporarily thermosoftenable layer having a uniform surface characteristic, said layer being at least 2 mils thick and comprising a hydrophobic thermoplastic resin, a thermosetting resin, a heat-activatable curing agent for said thermo-setting resin, and, uniformly distributed through said layer, a multitude of fine particles of a normally-dormant, heat-sensitive, puffing agent activatable at a temperature well above normal room temperature, and within approximately 150° F. of the thermosoftening temperature of said layer, to produce a gas as a result of chemical decomposition and thereby cause expansion of said layer under conditions of heat, said puffing agent being present in an amount sufficient to provide on rapid and complete heat activation of said layer an increase of at least 2 mils in the thickness thereof, and said layer being hardenable in expanded condition to an extent to support pressures at least on the order of 250 p. s. i. for about 15 seconds while maintaining areas of maximum expansion at least approximately 2 mils greater than the initial thickness thereof.

28. The sheet material of claim 27 wherein the puffing agent is present in an amount between about 1 and 10 percent by weight of the selectively-thermoexpansible layer.

29. The sheet material of claim 28 wherein the selectively-thermoexpansible layer contains a material which absorbs radiant energy, said sheet material being further characterized in that its layer is hardenable in expanded condition to an extent to support pressures at least on the order of 1000 p. s. i. for about 15 seconds while maintaining areas of maximum expansion at least approximately 2 mils greater than the initial thickness thereof.

U. S. DEPARTMENT OF COMMERCE  
PATENT OFFICE

**CERTIFICATE OF CORRECTION**

Patent No. 2,825,282      James B. Gergen et al.      March 4, 1958

It is hereby certified that error appears in the printed specification of the above numbered patent requiring correction and that the said Letters Patent should read as corrected below.

Column 13, line 73, for "100 p. s. i." read -- 1000 p. s. i. --; column 14, line 36, for "imbition" read -- imbibition --; column 17, line 33, for "flexile" read -- flexible --; line 56, for "have" read -- having --; line 74, for "patern" read -- pattern --.

Signed and sealed this 27th day of May 1958.

(SEAL)

Attest:  
KARL H. AXLINE  
Attesting Officer

ROBERT C. WATSON  
Commissioner of Patents